

Sept. 2, 1930.

D. E. WILLARD

1,774,687

PROCESS OF METAL CASTING

Filed Nov. 7, 1927



Inventor  
Donald E. Willard

By Barnard & Human  
Attorneys

## UNITED STATES PATENT OFFICE

DONALD E. WILLARD, OF DANVILLE, ILLINOIS

## PROCESS OF METAL CASTING

Application filed November 7, 1927. Serial No. 231,615.

My invention relates to the manufacture of metal castings having inserts of a different metal therein and more particularly to the manufacture of cast iron wheels, such as are employed on trucks, in which the hub has a steel insert therein in which the keyway by which the hub is secured to the axle is formed. Heretofore it has been difficult or impossible to secure satisfactory castings with inserts, particularly where the inserts are of substantial size, because of the chilling effect of the inserts on the molten metal when the latter is poured into the molds, the tendency of the two metals to separate during the cooling of the cast metal and the severe strain upon the structure set up during the cooling and shrinking of the casting, which often results in more or less serious cracking of the cast article. Often the cracks so formed cannot be detected until after heat treatment and sometimes until after the casting has been put in service. By the process of my invention which forms the subject of this application, I am able to produce castings with inserts, and more particularly cast iron wheels with steel hub linings in which there is a firm union between the insert and the cast metal.

In carrying out my improved process as applied to the manufacture of wheels of the character mentioned, I prepare a steel insert of suitable length to form the lining member for the hub and of a substantially less external diameter than the hub of the wheel to be cast, the insert having a central bore, which may be of approximately the diameter of the shaft to which the wheel is to be attached and transverse opening or passages from the bore through the wall of the insert. The mold in which the wheel is to be cast is prepared in the usual manner by means of a pattern with a cavity conforming to the wheel to be cast and also with an additional cavity or well communicating with the latter and adapted to contain a relatively large amount of metal. The insert is properly centered and mounted in the mold with its axis vertical and the molten cast iron, which is commonly malleable metal, is poured into the mold through the hollow of the insert.

The fluid metal flowing through the insert rapidly heats the latter. During the early stages the inflowing metal loses a considerable portion of its heat to the insert, but this portion of the mold charge mainly finds its way into the well prepared for it as previously mentioned. After the well is substantially full, as the flow continues the cast metal fills the bore of the insert and flows through the lateral or transverse passages to the exterior of the insert and into the mold cavity proper where it sets. In the meantime the insert has been heated to approximately the temperature of the cast metal and has been well watched by the latter so that a firm union of the metal of the insert and the cast metal is secured and the two metals are at substantially the same temperature during the cooling period with the result that the cracking and separation of the metals, mentioned above, is practically or entirely avoided. After the casting has cooled the surplus metal of the sprue and the bob formed in the well are removed and the cast metal drilled from the bore of the insert.

In the accompanying drawing and in the following specification I have shown and described a mold and preferred method for carrying out my invention and in the following claims have defined the invention with the purpose of claiming it as broadly as the prior art will permit.

In the drawings Fig. 1 is a fragmentary vertical section through a mold with a finished casting therein and also showing the lines of flow of the molten metal;

Fig. 2 is a fragmentary view of a wheel, partly in transverse section, formed according to my invention; and

Fig. 3 is a perspective of the insert in diametric section and on an enlarged scale.

In practicing my invention for the production of a malleable cast iron wheel with a steel insert lining, I form the mold and the cavity thereof in the usual manner. The molding cavity proper may be formed by means of a pattern designed to produce the required shape of wheel, the sand of the mold being illustrated at 5, 6. The central bottom portion of the wall of the mold cavity, how-

ever, is formed by a gate or core 13 supported in the sand of the cope and the upper surface of which conforms to the desired shape of the wheel. The gate or core 13 is, moreover, 5 formed with spaced openings or passages 14 and the sand 5, of the cope with a well 15 with which said passages communicate. Suitable sand cores 11 are supported in the mold to form the hollows of the spokes 12 of the 10 wheel.

15 The insert 7, which may be of soft steel, is shown as cylindrical in shape and of diameter less than that of the hub of the finished wheel but sufficient to provide for a bore 8 to receive the axle shaft and a sufficient wall thickness to permit a keyway 20 (see dotted line Figs. 1 and 2) for the spline to secure the wheel to the axle, to be formed therein. The 20 insert is also formed with transverse perforations or holes 9, the outer ends of which are countersunk as at 10. The insert is or may be supported on the gate or core 13 and centered with respect to the mold cavity before the cast metal is teemed.

25 The mold is centrally gated and the molten cast iron of which the body of the wheel, including the spokes, is to be formed, is poured through the bore of the insert. The insert is rapidly heated by the hot fluid metal and the latter is more or less cooled during the initial 30 heating.

35 The first part of the metal entering the mold, however, and a considerable proportion of the entire charge passes through the opening 14 in the gate or core 13 and into the well or sump 15 beneath the mold cavity proper, so that it is immaterial that this metal is partially cooled. After the well is filled, the insert in the meantime having been highly 40 heated as above explained, the pouring is continued and the freshly poured metal fills the lower portion of the bore of the insert and then overflows through the opening 9 into the mold cavity proper about the insert 45 and forms the spokes and the main portion of the hub of the wheel. Since the insert is heated to approximately the temperature of the fluid metal it no longer chills the latter and thus defective castings are largely avoided. Pouring is continued until the 50 mold and gate 16 are substantially full. The casting is now permitted to cool and the insert cools with the cast metal. Cooling is relatively slow, however, because of the body 55 of hot metal contained in the sump. By reason of the act that the insert is highly heated before the metal with which it is to be surrounded is in contact therewith and then cools along with the cast metal, it forms a firm 60 union with the latter and separation of the metal and cracking during or after cooling are largely avoided.

65 After the casting has sufficiently cooled it is withdrawn from the mold, the bob or mass of metal formed in the well and the sprue

separated therefrom. The insert is then bored out and reamed to receive the axle and the keyway machined therein. If the original bore of the insert is of proper diameter it is sufficient to remove the cast metal therefrom. Ordinarily, however, the bore 8 as originally formed is too small and in drilling and reaming a portion of the metal of the insert is removed as indicated in dotted lines at 18, Fig. 1. In the completed wheel the 70 insert and casting are held together not merely by the adhesion of the metals as previously explained, but also by reason of the cast metal cores extending into the openings 9 in the insert.

75 I claim:

1. A wheel for trucks and the like comprising a cast metal hub and spokes and a steel insert liner having an axial bore therein to receive an axle and transverse openings 80 into which the metal of the casting extends.

2. A method of casting an iron article having a tubular insert therein which consists in forming a mold having a molding cavity proper and a well beneath and connected thereto, forming an insert with a central bore and transverse bores, supporting the insert substantially centrally of the mold cavity and with its central bore in communication with the well in the mold and teeming molten 90 cast metal through the bore of the insert into the well and through said bore and the transverse bores of the insert into the mold cavity about the insert.

DONALD E. WILLARD.

100

105

110

115

120

125

130